

## UNITED STATES PATENT OFFICE.

LEONARD E. BRANCHEN, OF ROCHESTER, NEW YORK, ASSIGNOR TO EASTMAN KODAK COMPANY, OF ROCHESTER, NEW YORK, A CORPORATION OF NEW YORK.

## PROCESS OF REDUCING THE VISCOSITY CHARACTERISTICS OF NITROCELLULOSE.

No Drawing.

Application filed September 1, 1925. Serial No. 53,951.

This invention relates to processes for reducing the viscosity characteristics of nitrocellulose. One object of the invention is to provide a simple and inexpensive process for reducing said viscosity characteristics safely and within a short time. A further object of the invention is to provide a process for reducing rapidly and accurately the viscosity characteristics of nitrocellulose when it is in the solid colloidized state, and even when mixed with high-boiling organic compounds or softeners. Another object is to provide a process which can be operated at atmospheric pressure and room temperature. Still a further object is to provide a process in which a series of baths are used in such a way that the material of the first bath can be used repeatedly without contamination by the second bath. Another object of the invention is to provide a process in which the nitrocellulose is converted into such a state that the acids, which lower the viscosity, can be very easily and quickly washed out of the nitrocellulose. Still another object of the invention is to provide a process in which the nitrocellulose remains substantially undissolved, thereby avoiding unnecessary and troublesome precipitation steps. Other objects will hereinafter appear.

It is highly desirable, when making solutions of nitrocellulose for spraying to have a high concentration of nitrocellulose and yet to keep the viscosity of the solutions at a low point. In order to obtain such solutions from the nitrocelluloses which have high viscosity characteristics, it is necessary to modify the latter. The kinds of nitrocellulose which are found in pyroxylin waste and film scrap, and similar waste materials, are nearly always of the high-viscosity species. It is, therefore, desirable to provide a suitable process for lowering the viscosity characteristics of nitrocellulose, particularly when the latter is in solid colloidized form, and associated with high-boiling compounds, like camphor and butyl alcohol, in inexpensive or waste materials.

I have found that a process of this kind can be carried out by first softening the nitrocellulosic material with a suitable liquid and thereafter treating it with an aqueous acid solution. The softening step makes the nitrocellulosic material more susceptible to the action of the acid and thereby shortens the time for producing the desired reduction.

Moreover, it makes such reduction more uniform throughout the mass of material. It is a surprising fact that the condition which is created in the nitrocellulose by the preliminary softening treatment, persists not only throughout the subsequent treatment with acid, but likewise exists during the final washing operations.

Various penetrant liquids may be employed such, for instance, as one that merely softens the nitrocellulosic material, like films, and has a solvent action on the high-boiling organic compounds therein, such as camphor, butyl alcohol, triphenyl phosphate, tricresyl phosphate, monochlornaphthalene and the like. It is sometimes useful to control the action of an especially strong penetrant by diluting it with water, so that it merely softens the nitrocellulose, the action being always stopped before the nitrocellulose itself is dissolved to any substantial extent.

The operations may be carried out at room temperature and atmospheric pressure. Various acids may be employed in the second step of the process in which the viscosity is reduced. I may for example employ a nitric acid bath, especially one containing oxides of nitrogen as indicated in copending application, Serial No. 12,181, C. U. Prachel, filed Feb. 27, 1925, for process of treating nitrocellulosic materials.

I shall now describe one embodiment of my invention, but it will be understood that the latter is not restricted to the details of this illustration except as indicated in the appended claims. The nitrocellulosic material is preferably comminuted. Solid colloidized nitrocellulose, such as pyroxylin waste, or film scrap from which the gelatinous coatings have been removed, is chopped up into small pieces.

The comminuted material is then treated by the penetrant liquid, say a bath of methyl alcohol toned down by 5% of water. The material is allowed to soften in contact with this liquid, say by being immersed in it, for 1 to 5 hours at room temperature and atmospheric pressure. A slight heating is permissible to shorten the time of treatment. Thus I may conduct the above operations at 40° C. and stop the action in about two hours. The action in all forms of my process is stopped before any substantial dissolving of the nitrocellulose takes place, and

before the pieces of nitrocellulosic material gum together into an unmanageable mass. This initial leaching step softens the material and leaches out some of the high-boiling 5 organic compounds which are present with the nitrocellulose. It opens up the latter to subsequent treatment to a surprising degree.

When the pre-leaching step is completed, the nitrocellulosic material is separated from 10 the leaching bath, say by lifting the particles of the nitrocellulosic material out of the bath and draining them, or running the bath off into another receptacle, and squeezing out the excess of liquid. This maintains 15 the bath in a form free from acid and free from deterioration by the formation of compounds which would be created if acid remained in the bath for a considerable time.

The nitrocellulose, in its highly suscepti- 20 ble condition from the first treatment, is then brought into contact with an acid bath to reduce its viscosity characteristics. The acid bath may conveniently be a 30% aqueous solution of spent mixed acids from 25 a cellulose nitrating plant. Such a solution may include approximately 20%  $H_2SO_4$ , 10%  $HNO_3$ , and 1 to 2% of nitrogen oxides, say  $N_2O_4$ . Of course, there is nothing critical about these proportions, and they may 30 be varied widely without departing from the invention. In fact, other well known acids and acid mixtures may be substituted. I have found the above mixture, however, 35 to be preferable because it acts rapidly and safely at room temperature and has a bleaching tendency which makes other bleaching action practically unnecessary.

The treatment may take place in any suitable acid-resisting container, the pieces of 40 nitrocellulosic material being immersed in the liquid. By conducting the operations at room temperature, the loss of valuable oxides of nitrogen is reduced to a minimum, even when the soaking in the acid lasts for 45 several days. Of course, the vessels may be covered.

The duration of the treatment is controlled by tests. When samples show that 50 the desired degree of low viscosity has been reached, the acid and nitrocellulose are separated, say by draining off the acid from the material, preferably assisted by pressure on the latter.

Finally the nitrocellulosic material is 55 washed with successive changes of water. The latter may be heated, if desired to hasten the action, say to about 75° C. But by reason of the opening up of the nitrocellulose by my pre-treatment, the acid can be 60 relatively quickly washed out by successive changes of cold water or water at room temperature. The increased thoroughness with which the washing can be carried out, because of the susceptible condition of the 65 nitrocellulose, results in a very noticeably

improved stability of the product when subjected to the usual heat tests.

The concentration of the mixed acids in the second step of the process can be altered considerably. Instead of mixed acids, I may 70 use a single acid, say for instance nitric acid containing some nitrogen oxides. A 6% aqueous solution of nitric acid containing 1.2% of nitrogen oxides has been demonstrated, for example, to operate effectively 75 at room temperature during a treatment of a few days. In general the preferred baths contain from 5 to 2% of  $HNO_3$ , 10 to 30% of  $H_2SO_4$  and 1/2 to 10% of nitrogen oxide.

While I prefer to use in the first step of 80 the process an active nitrocellulosic solvent, toned down by water to the point where it acts merely as a penetrant, I may employ other penetrants which have little, if any, solvent action on the nitrocellulose such as 85 ethyl alcohol.

Having thus described my invention, what I claim as new and desire to secure by Letters Patent is:

1. The process of treating nitrocellulose, 90 which comprises first softening it with a penetrant liquid to make it more susceptible to subsequent treatment, and thereafter acting on it separately with an aqueous acid solution until the viscosity characteristics of the nitrocellulose are reduced.

2. The process of treating solid colloidized 100 nitrocellulose associated with a high-boiling organic compound, which comprises first softening it with a penetrant liquid, which has a solvent action on said organic compounds, and thereafter acting on said material with an aqueous acid solution until the viscosity characteristics of the nitrocellulose are reduced.

3. The process of treating solid colloidized 110 nitrocellulose material, which comprises softening it with a penetrant liquid containing water and an active nitrocellulose solvent, stopping the action of said liquid before the nitrocellulose is dissolved, and thereafter acting on it with an aqueous acid solution until the viscosity characteristics of the nitrocellulose are reduced.

4. The process of treating solid colloidized 115 nitrocellulose associated with a high-boiling organic compound, which comprises softening it with a mixture of water and methyl alcohol to make it more susceptible to subsequent treatment, stopping the action before the nitrocellulose is dissolved, and thereafter acting on it with an aqueous acid solution until the viscosity characteristics of the nitrocellulose are reduced.

5. The process of treating solid colloidized 120 nitrocellulose, which comprises acting thereon with a penetrant liquid, the action being stopped before the nitrocellulose is dissolved, separating said liquid from the 130 nitrocellulosic material, and thereafter act-

ing on it with an aqueous acid solution until the viscosity characteristics of the nitrocellulose are reduced.

6. The process of treating solid colloidized nitrocellulose, which comprises softening it with a penetrant liquid to facilitate subsequent treatment, separating the bulk of said liquid from said nitrocellulose, and thereafter acting on it with an aqueous acid solution containing oxides of nitrogen until the viscosity characteristics of the nitrocellulose are reduced.

7. The process of treating solid colloidized nitrocellulose associated with a high-boiling organic compound, which comprises first treating it with a penetrant liquid until its susceptibility to subsequent liquid treatments is increased, separating said penetrant liquid from said nitrocellulose, acting on said nitrocellulose with an aqueous acid solution

until the viscosity characteristics of the nitrocellulose are reduced, removing the bulk of said acid solution from the nitrocellulose and washing the latter to remove residual acid from it.

8. The process of treating solid colloidized nitrocellulose associated with a high-boiling organic compound, which comprises first leaching it with a penetrant liquid which has a solvent action on said organic compound, separating the bulk of said liquid from said nitrocellulose, treating said nitrocellulose with an aqueous acid solution until its viscosity characteristics are reduced, and removing and washing out the acid from said nitrocellulose.

Signed at Rochester, New York, this 24th day of August, 1925.

LEONARD E. BRANCHEN.